

## UNITED STATES PATENT OFFICE

2,385,763

## PHOTOGRAPHIC DEVELOPERS

Verne H. Reckmeyer, Binghamton, N. Y., assignor  
to General Aniline & Film Corporation, New  
York, N. Y., a corporation of Delaware

No Drawing. Application May 19, 1942,  
Serial No. 443,559

4 Claims. (Cl. 95—88)

This invention pertains to a photographic developer, and more particularly to a developer which has greatly improved characteristics of speed and fineness of grain.

Many so-called fine grain developers have been proposed from time to time in the past, but none of these prior developers is entirely satisfactory. In all of these previous proposals, improved fineness of grain is achieved only at the cost of a considerable loss in effective threshold speed. Attempts have been made to avoid this speed loss by the use of various alkalies in the developer. The use of the customary alkalies, such as borax, sodium metaborate, trisodium phosphate, triethanol amine and the like, however, has always resulted in a considerable coarsening of the grain. Thus the desirable fine grain characteristics were lost.

With these defects of the prior art in view, it is accordingly one object of the present invention to provide a new and improved fine grain developer.

A further object is to provide a fine grain developer which will retain threshold speed without impairment of the fine grain characteristics.

Still another object is to provide a deep working fine grain developer which will maintain maximum speed with a minimum of graininess.

Other objects and advantages will be apparent from the following description.

It is known that in the use of ordinary developers in connection with photographic gelatino silver halide emulsions, the main development takes place nearest to the surface of the exposed layer. In other words, the chief density is due to the presence of developed silver particles near this surface. These silver particles form grain clusters, and it is apparent that the presence of these grain clusters in a relatively thin layer near the surface of the emulsion will give rise to a graininess effect due to passage of light between the grains.

To avoid the above difficulties, certain developers have been used which achieve the same given density by a more uniform distribution of silver throughout the light sensitive layer. These are the so-called deep working developers, of which para-phenylene diamine is typical. They show a less noticeable graininess effect since the developed silver particles are more evenly distributed in depth and the particles in one layer tend to block up the openings between the developed silver particles in other layers.

In these deep working developers, however, the top layer of silver particles is often dissolved out

by reason of the characteristic solvent action of the developing compound. Thus, even though the graininess characteristics are improved, the developer is unsatisfactory from a practical standpoint due to the effective loss in speed, which may correspond to differences of from 1 to 1½ lens stops in a particular case.

We have now found that the above stated objects can be accomplished by the use of a developing agent to give uniform distribution of the developed silver particles energized with an easily oxidizable organic compound, which, when oxidized, tends to set free a limited amount of alkali. Preferably easily oxidizable alkali metal salts of organic compounds of the phenolic type are employed for this purpose. Thus, the phenolates are particularly useful as energizers. If the developing agent employed were energized by ordinary alkalies the increased clustering or coarseness of grain typical of prior art developers would result.

Typical examples of the easily oxidizable compounds according to the present invention are the alkali metal salts of compounds of the N-substituted o-amino phenols such as the alkali metal salts of 2(di(hydroxyethyl) 1-amino-1-hydroxy benzenes disclosed in U. S. Patent 1,712,716 of Gustav Reddelien and Werner Mueller. These salts are characterized by their sensitivity to oxidation and by the fact that, when so oxidized, they set free a limited amount of alkali. These compounds have a weak developing action by themselves but such developing action must be weaker than that of the developing agent which the easily oxidizable compound energizes. Thus, when mono N-methyl o-amino phenol is the developing agent the energizer such as 2(di(hydroxyethyl) 1-amino-1-hydroxy benzene has a weaker developing action. The effect of the energizer to set free a limited amount of alkali, results in an increase in speed without any appreciable increase in grain. It should be noted that the improved results of the present invention as to fineness of grain with increased threshold speed, which are not achieved by the use of customary sources of alkali, can be determined by measuring the fineness of grain on a graininess meter.

As the developing agent itself, we use mono N-alkyl o-amino phenols. Especially good results are obtained by the use of monomethyl ortho amino phenol. As a matter of fact, the addition of a substantial amount of hydroquinone to the ortho-methyl amino phenol is desirable in order to obtain greatly improved contrast characteristics. While the use of hydroquinone has been

proposed previously in combination with ortho-methyl amino-phenols, it has not been proposed in the threefold combination of a mono-N-alkyl ortho amino phenol, hydroquinone, and an energizer of the type described above. The new developers which include these three ingredients are particularly important because of the extreme fineness of grain which is characteristic of the resulting developed image. This fineness of grain is achieved without loss in threshold speed. In fact, the threshold speed can even be increased by the use of larger amounts of the energizing compounds.

The following examples will serve to illustrate the invention. The parts are by weight unless otherwise indicated.

*Examples*

|                                                                                                                                                                    | Grams |
|--------------------------------------------------------------------------------------------------------------------------------------------------------------------|-------|
| I. Sodium sulfite                                                                                                                                                  | 100.0 |
| o-Methyl aminophenol                                                                                                                                               | 5.0   |
| 2[Di(hydroxyethyl)] - amino-1-hydroxy benzene sodium salt                                                                                                          | 4.0   |
| Hydroquinone                                                                                                                                                       | 7.5   |
| Water is added to make the solution up to                                                                                                                          | 25    |
| 1000 cc. This solution will develop 35 mm. film of the type sold by the General Aniline & Film Co. under the trade name "Supreme," in from 12-18 minutes at 68° F. |       |
| II. Sodium sulfite                                                                                                                                                 | 100.0 |
| o-Methyl amino phenol                                                                                                                                              | 5.0   |
| 2[Di(hydroxyethyl)] - amino - 1 - hydroxy benzene sodium salt                                                                                                      | 4.0   |

Water is added to make the solution up to 35

1000 cc. This solution will develop 35 mm. film of the type mentioned in Example I, in from 20-30 minutes at 68° F.

Having now fully set forth and described my invention, and having illustrated the best manner in which to perform it by specific examples, what I claim as new and desire to have secured by Letters Patent is:

1. A photographic developer comprising in combination an N-mono alkyl o-amino phenol, and an alkali metal salt of a 2[di(hydroxyethyl)]-1-amino-1-hydroxy benzene which upon oxidation sets free limited amounts of alkali said developer being initially free of alkali.

2. A photographic developer comprising in combination hydroquinone an N-mono alkyl o-amino phenol, and an alkali metal salt of a 2[di(hydroxyethyl)]-1-amino-1-hydroxy benzene which upon oxidation sets free limited amounts of alkali said developer being initially free of alkali.

3. A photographic developer comprising in combination hydroquinone, o-methyl amino-phenol, and the sodium salt of 2[di(hydroxyethyl)]-amino-1-hydroxy benzene which upon oxidation sets free limited amounts of alkali said developer being initially free of alkali.

4. A photographic developer comprising in combination o-methyl amino-phenol and the sodium salt of 2[di(hydroxyethyl)]-amino-1-hydroxy benzene which upon oxidation sets free limited amounts of alkali said developer being initially free of alkali.

VERNE H. RECKMEYER.

CERTIFICATE OF CORRECTION.

Patent No. 2,385,763.

September 25, 1945.

VERNE H. RECKMEYER.

It is hereby certified that error appears in the printed specification of the above numbered patent requiring correction as follows: Page 2, second column, line 12, claim 1, for "-1-amino-1-" read -- -amino-1- --; and that the said Letters Patent should be read with this correction therein that the same may conform to the record of the case in the Patent Office.

Signed and sealed this 26th day of February, A. D. 1946.

Leslie Frazer

First Assistant Commissioner of Patents.

(Seal)

proposed previously in combination with ortho-methyl amino-phenols, it has not been proposed in the threefold combination of a mono-N-alkyl ortho amino phenol, hydroquinone, and an energizer of the type described above. The new developers which include these three ingredients are particularly important because of the extreme fineness of grain which is characteristic of the resulting developed image. This fineness of grain is achieved without loss in threshold speed. In fact, the threshold speed can even be increased by the use of larger amounts of the energizing compounds.

The following examples will serve to illustrate the invention. The parts are by weight unless otherwise indicated.

*Examples*

|                                                                                                                                                                    | Grams |
|--------------------------------------------------------------------------------------------------------------------------------------------------------------------|-------|
| I. Sodium sulfite.....                                                                                                                                             | 100.0 |
| o-Methyl aminophenol.....                                                                                                                                          | 5.0   |
| 2[Di(hydroxyethyl)] - amino-1-hydroxy benzene sodium salt.....                                                                                                     | 4.0   |
| Hydroquinone.....                                                                                                                                                  | 7.5   |
| Water is added to make the solution up to                                                                                                                          | 25    |
| 1000 cc. This solution will develop 35 mm. film of the type sold by the General Aniline & Film Co. under the trade name "Supreme," in from 12-18 minutes at 68° F. |       |
| II. Sodium sulfite.....                                                                                                                                            | 100.0 |
| o-Methyl amino phenol.....                                                                                                                                         | 5.0   |
| 2[Di(hydroxyethyl)] - amino - 1 - hydroxy benzene sodium salt.....                                                                                                 | 4.0   |

Water is added to make the solution up to 35

1000 cc. This solution will develop 35 mm. film of the type mentioned in Example I, in from 20-30 minutes at 68° F.

Having now fully set forth and described my invention, and having illustrated the best manner in which to perform it by specific examples, what I claim as new and desire to have secured by Letters Patent is:

1. A photographic developer comprising in combination an N-mono alkyl o-amino phenol, and an alkali metal salt of a 2[di(hydroxyethyl)]-1-amino-1-hydroxy benzene which upon oxidation sets free limited amounts of alkali said developer being initially free of alkali.

2. A photographic developer comprising in combination hydroquinone an N-mono alkyl o-amino phenol, and an alkali metal salt of a 2[di(hydroxyethyl)]-1-amino-1-hydroxy benzene which upon oxidation sets free limited amounts of alkali said developer being initially free of alkali.

3. A photographic developer comprising in combination hydroquinone, o-methyl amino-phenol, and the sodium salt of 2[di(hydroxyethyl)]-amino-1-hydroxy benzene which upon oxidation sets free limited amounts of alkali said developer being initially free of alkali.

4. A photographic developer comprising in combination o-methyl amino-phenol and the sodium salt of 2[di(hydroxyethyl)]-amino-1-hydroxy benzene which upon oxidation sets free limited amounts of alkali said developer being initially free of alkali.

VERNE H. RECKMEYER.

CERTIFICATE OF CORRECTION.

Patent No. 2,385,763.

September 25, 1945.

VERNE H. RECKMEYER.

It is hereby certified that error appears in the printed specification of the above numbered patent requiring correction as follows: Page 2, second column, line 12, claim 1, for "-1-amino-1-" read -- -amino-1- --; and that the said Letters Patent should be read with this correction therein that the same may conform to the record of the case in the Patent Office.

Signed and sealed this 26th day of February, A. D. 1946.

Leslie Frazer

First Assistant Commissioner of Patents.

(Seal)